

## UNITED STATES PATENT OFFICE

2,157,383

## LEAD ALLOY

François Cuveilliez, Hoboken, near Antwerp, Belgium, assignor to Société Générale Métallurgique de Hoboken, Hoboken, near Antwerp, Belgium

No Drawing. Application August 2, 1938, Serial No. 222,670. In Great Britain October 15, 1937

## 1 Claim. (Cl. 75—166)

This invention relates to lead alloys to be used in the chemical industry.

A lead alloy according to the present invention is of the usual compact, non-porous, structure, and comprises from 0.3 to 13% Sb and from 0.2 to 5% Hg.

Moreover, the alloy may contain one or more of the metals Zn, Ca, Bi:

|       | Per cent |
|-------|----------|
| 10 Zn | 0 to 0.6 |
| Ca    | 0 to 0.1 |
| Bi    | 0 to 1   |

The non-porous alloys according to the present invention not only resist corrosion by chemical agents, more particularly of sulphuric acid and nitrous gases, as is the case with sulphuric acid plants of the chamber method type, but in addition they have also a high resistance to mechanical and physical efforts.

Example of an alloy according to the invention:

|    | Per cent |
|----|----------|
| Sb | 3        |
| Hg | 0.75     |
| Zn | 5        |

The rest: Pb.

The alloy according to the present invention has a compact structure, such as industrial alloys generally have when they are made by the known processes of casting, moulding or rolling.

## I claim:

A compact lead alloy, to be used more particularly against corrosion by chemical agents, consisting of from 0.3 to 13% of antimony, from 0.2 to 5% of mercury, and lead for the rest.

FRANÇOIS CUVEILLIEZ. 20